# EUROPEAN PATENT SPECIFICATION

(11) **EP 2 045 022 B1**
(45) Date of publication and mention of the grant of the patent: **30.10.2019**
(21) Application number: 08172622.6
(22) Date of filing: 28.05.2004
(51) Int. Cl.: B05D 5/06, B05D 7/00

(54) **Method for forming brilliant coating film and coated article showing metallic effect**
Verfahren zum Bilden eines Glanzbeschichtungsfilm und beschichteter Artikel mit Metalleffekt
Procédé de formation d'un film de revêtement brillant et article revêtu doté d'un effet métallique

(30) Priority: 30.05.2003 JP 2003155609; 30.05.2003 JP 2003155610; 30.05.2003 JP 2003155611
(43) Date of publication of application: 08.04.2009
(62) Divisional of application: 04735373.5
(73) Proprietor: Honda Motor Co., Ltd., Minato-ku Tokyo 107-8556 (JP); Nippon Paint Automotive Coatings Co., Ltd., Osaka 573-1153 (JP)
(72) Inventor: Ogawa, Takeshi, SAITAMA 351-0193 (JP); Ihara, Satoru, SAITAMA 351-0193 (JP); Uchiyama, Toshihiko, OSAKA 573-1153 (JP); Inoue, Masanobu, OSAKA 573-1153 (JP); Miyazoe, Seigo, TOKYO 140-8675 (JP); Shiraga, Ryuichi, TOKYO 140-8675 (JP)
(74) Representative: Cabinet Plasseraud

(56) References cited:
- WO-A1-97/30795
- DE-A- 4 418 490

## Description

### Technical Field

The present invention relates to a method for forming a brilliant coating film and an article coated with the brilliant coating film.

### Related Art

Brilliant coating compositions containing aluminum or mica flakes have been used for forming metallic coating films with metallic luster.

Methods for forming the brilliant coating films using the brilliant coating compositions include a method described in JP-A-2002-35688 of forming a metallic coating film excellent in orientation, density, flip-flop property, brilliantness, etc. In this multilayer film-forming method, a heat-curable base coating composition containing a hydrophilic organic solvent and water is applied to a substrate, the solid content of the surface of the applied composition is controlled to 70% by mass or more without curing the applied composition, a metallic coating composition containing a hydrophilic organic solvent is applied to the surface, and a clear coating composition is further applied if necessary.

However, the method of JP-A-2002-35688 requires measures against environmental affect of VOCs (volatile organic compounds) because the metallic coating composition containing a hydrophilic organic solvent as the second base coating composition contains only organic solvents without water. Further, the method comprises the step of preheating the applied heat-curable base coating composition to control the solid content to 70% by mass or more without curing the composition, whereby the method needs complicated lines with a preheating unit in a base coating zone.

Accordingly, an object of the present invention is to provide a method that can form a brilliant coating film with an excellent brilliant appearance by using aqueous first and second base coating compositions without preheating the applied first base coating composition, and a coated article having the brilliant coating film.

### Summary of The Invention

As a result of intense research, the inventors have accomplished the present invention. More specifically, the following is provided.
1. A method for forming a brilliant coating film on a substrate, comprising in sequence the steps of:
   (1) applying an aqueous first brilliant base coating composition to the substrate to form a first base coating at a first stage in a base coating zone;
   (2) applying an aqueous second brilliant base coating composition to the first base coating obtained in the step (1) to form a second base coating at a second stage in the base coating zone;
   (3) applying a clear coating composition to the second base coating obtained in the step (2) to form a clear coating in a clear coating zone; and
   (4) simultaneously heating the uncured coatings formed in the steps (1), (2) and (3) to cure the coatings,
      with the following provisos II, and III:
      the proviso II of a condition (A-2) that the aqueous first brilliant base coating composition has a brilliant pigment mass concentration of 3 to 25 % and the aqueous second brilliant base coating composition has a brilliant pigment mass concentration of 7 to 30%, and a condition (B-2) that the ratio of the brilliant pigment mass concentration of the aqueous first brilliant base coating composition to the brilliant pigment mass concentration of the aqueous second brilliant base coating composition is 1/3,5 to 1/1,5; and
      the proviso III of a condition (A-3) that the aqueous first brilliant base coating composition comprises at least one organic solvent and water, and the mass ratio of the at least one organic solvent to the water is from 5/95 to 49/51, and a condition (B-3) that the at least one organic solvent used in the aqueous first brilliant base coating composition contains 40 to 100% by mass of a particular organic solvent, which has a solubility parameter of 9,7 to 14.5 and an evaporation rate of 200 to 750 when n-butyl acetate has an evaporation rate of 100 at 25°C
         and which is acetane, methyl alcohol, ethyl alcohol or isopropyl alcohol.
         the first base coating obtained in the step (1) to form a second base coating at and
      the aqueous first base coating having a dry film thickness of 5 to 15 µm
      the aqueous second base coating having a dry film thickness of 2 to 8 µm
      the ratio of the dry film thickness of the first base coating to the dry film thickness of the second base coating being 1.5/1 to 5/1 and
      the clear coating film having a dry film thickness of 10 to 60 µm.

   Document WO97/30795 specifically discloses at Examples 3a-c a method for forming a brilliant film on a substrate, said method comprising the successive steps of:
   - applying an aqueous first base coating composition containing a brilliant pigment (aluminium bronze) to the substrate to form a first base coating, and
   - applying an aqueous second base coating composition containing the same brilliant pigment to the substrate to form a second base coating.

   However the method disclosed in WO97/30795 does not show contrary to the present invention:
   a brilliant pigment concentration of the second coating composition (PWC2) ranging from 7% to 30%.
   a ratio between the brilliant pigment concentration of the first coating composition (PWC1) and the brilliant pigment concentration of the second coating composition (PWC2), between 1/3.5 and 1/1.5;
   and an amount of organic solvent selected in the group formed by the acetone, methyl alcohol, ethyl alcohol and isopropyl alcohol ranging from 40 to 100% by mass of the total amount of organic solvents used in the first brilliant base coating composition (condition B-3).
2. The method for forming a brilliant coating film according to 1 wherein the method satisfies a condition (C) that the aqueous second brilliant base coating composition comprises at least one organic solvent and water, and the mass ratio of the at least one organic solvent to the water is from 5/95 to 49/51.
3. The method for forming a brilliant coating film according to 1 or 2 wherein the aqueous second brilliant base coating composition contains 0.1 to 5 parts by mass of a fluorine- or silicone-based additive per 100 parts by mass of the vehicle solid contents.
4. A coated article comprising a brilliant coating film formed by the method according to any one from 1 to 4.

### Best Mode for Carrying Out The Invention

Constituents of the present invention are described in detail below.

### First method for forming a brilliant coating film

A first method according to an embodiment of the present invention for forming a brilliant coating film comprises in sequence the steps of (1) applying an aqueous first brilliant base coating composition to a substrate to form a first base coating at a first stage in a base coating zone; (2) applying an aqueous second brilliant base coating composition to the first base coating formed in the step (1) to form a second base coating at a second stage in the base coating zone; (3) applying a clear coating composition to the second base coating formed in the step (2) to form a clear coating in a clear coating zone; and (4) simultaneously heating the uncured coatings formed in the steps (1), (2) and (3) to cure the coatings, with the following provisos II, and III, and optionally with proviso I.

### Proviso I

The proviso I is that the conditions (A-1) and (B-1) are satisfied. The condition (A-1) is that the aqueous first brilliant base coating composition has a solid content of 10 to 45% by mass and the aqueous second brilliant base coating composition has a solid content of 10 to 40% by mass. The condition (B-1) is that the ratio of the solid content of the aqueous first brilliant base coating composition to the solid content of the aqueous second brilliant base coating composition is from 1.1/1 to 4/1.

### Proviso II

The proviso II is that the conditions (A-2) and (B-2) are satisfied. The condition (A-2) is that the aqueous first brilliant base coating composition has a brilliant pigment mass concentration (hereinafter referred to as "PWC") of 3 to 25% and the aqueous second brilliant base coating composition has a brilliant pigment PWC of 7 to 30 %. The condition (B-2) is that the ratio of the brilliant pigment PWC of the aqueous first brilliant base coating composition to the brilliant pigment PWC of the aqueous second brilliant base coating composition is 1/3,5 to 1/1,5.

### Proviso III

The proviso III is that the conditions (A-3) and (B-3) are satisfied. The condition (A-3) is that the aqueous first brilliant base coating composition comprises a solvent containing at least one organic solvent and water, and the mass ratio of the at least one organic solvent to the water is from 5/95 to 49/51. The condition (B-3) is that the at least one organic solvent used in the aqueous first brilliant base coating composition contains 40 to 100% by mass of a particular organic solvent, which has a solubility parameter of 9.7 to 14.5 and an evaporation rate of 200 to 750 when n-butyl acetate has an evaporation rate of 100 at 25°C.

### Second method for forming brilliant coating film

A second method according to an embodiment of the present invention for forming a brilliant coating film is the first method with the condition (C) that the aqueous second brilliant base coating composition comprises a solvent containing at least one organic solvent and water, and the mass ratio of the at least one organic solvent to the water is from 5/95 to 49/51 .

### Third method for forming brilliant coating film

A third method according to an embodiment of the present invention for forming a brilliant coating film is of the first to or second methods, in which the aqueous second brilliant base coating composition contains 0.1 to 5 parts by mass of a fluorine- or silicone-based additive per 100 parts by mass of the vehicle solid content.

### Substrate

Materials for the substrate used in the methods according to an embodiment of the present invention for forming a brilliant coating film are not limited, but include metals such as iron, aluminum, copper, and alloys thereof; inorganic materials such as glass, cement, and concrete; plastic materials such as resin (e.g. polyethylene resin, polypropylene resin, ethylene-vinyl acetate copolymer resin, polyamide resin, acrylic resin, vinylidene chloride resin, polycarbonate resin, polyurethane resin, epoxy resin, etc.) and FRP (fiber-reinforced plastic); and natural or synthetic materials such as wood material and textile material (e.g. paper, cloths, etc.).

In the methods according to the embodiments of the present invention for forming a brilliant coating film, if a conductive substrate for a main body or parts of the automobile is employed, the substrate may be coated with an undercoating film (by a chemical treatment, an electrodeposition coating, etc.)or with an intermediate coating film in addition to such an undercoating film. If a non-conductive substrate for a main body or parts of the automobile is employed, the substrate may be coated with a primer after a chemical treatment and if necessary a conductive treatment.

The undercoating film acts to improve the adhesion of the brilliant coating film to the substrate, the property of hiding or covering or concealing the substrate, the anticorrosion property, and the rust preventive property. The undercoating film may be formed by applying, baking, and curing an undercoating composition. The undercoating film may have a dry film thickness of 8 to 30 µm. The undercoating composition is not particularly limited, but may include various kinds of compositions such as a cationic electrodeposition coating composition and an anionic electrodeposition coating composition. The electrodeposition coating composition is electrodeposited and cured by baking in a condition in accordance with the type of the composition.

The intermediate coating film may be formed on the substrate or on the undercoating film by applying an intermediate coating composition to improve the adhesion of the brilliant coating film to the substrate or the undercoating film, the property of hiding or covering or concealing the substrate or the undercoating film, and the chipping resistance. The intermediate coating film may have a dry film thickness of 10 to 50 µm. For example, the intermediate coating composition may be a composition containing a hydroxyl-containing polyester resin and/or a hydroxyl-containing acrylic resin, and a melamine resin and/or a blocked polyisocyanate. Such a composition is applied, and dried or cured at a room temperature or a baking temperature in accordance with the type of the composition.

In the methods for forming a brilliant coating film according to an embodiment of the present invention, the base coating zone is an area in which the base coatings are formed, and the base coatings are lower layers of the multilayered overcoating film.

In the methods for forming a brilliant coating film according to an embodiment of the present invention, the clear coating zone is an area in which the clear coating (or the clear top coating) is formed, and the clear top coating is an upper layer of the multilayered overcoating film.

In the methods for forming a brilliant coating film according to an embodiment of the present invention, the base coatings are successively formed in the base coating zone. The first base coating is formed at the first stage and the second base coating is formed at the second stage. In the embodiment of the present invention, it is important that different particular coating compositions are used respectively at the first and second stages.

### Step (1)

In the step (1) of the methods for forming a brilliant coating film according to an embodiment of the present invention, the first base coating is formed by applying the aqueous first brilliant base coating composition (which may be referred to as the aqueous first base coating composition) at the first stage in the base coating zone.

The aqueous first base coating composition contains an aqueous resin as a vehicle-forming resin. The aqueous resin can be made hydrophilic by controlling the acid value and by neutralizing the carboxyl groups (for example, 50% or more of the carboxyl groups) of the resin with a basic substance. In the embodiment of the present invention, the aqueous resin may include a water-soluble resin, a water-dispersible resin, and an emulsion resin. Examples of the basic substances include ammonia, methylamine, ethylamine, dimethylamine, diethylamine, trimethylamine, triethylamine, dimethylethanolamine, diethanolamine, triethanolamine, etc. More preferable among them are diethanolamine, dimethylethanolamine, and triethanolamine. The solvent for the aqueous first base coating composition may be composed mainly of water and may contain organic solvents.

For the vehicle-forming resin, an acrylic resin or a polyester resin may be used along with an amino resin and/or a blocked polyisocyanate and/or polycarbodiimide compound as a crosslinking agent for the resin. The acrylic resin is more preferably used for forming the base coating.

The acrylic resin may be a copolymer of acrylic monomers and other ethylenic unsaturated monomers. Examples of the acrylic monomers usable for the copolymer include acrylic or methacrylic ester such as methyl, ethyl, propyl, n-butyl, i-butyl, t-butyl, 2-ethylhexyl, lauryl, phenyl, benzyl, 2-hydroxyethyl, or 2-hydroxypropyl ester; amide group-containing acryl monomers such as acrylamide, methacrylamide, N,N-dimethylacrylamide, N,N-dimethylmethacrylamide, N,N-dibutylacrylamide, and N,N-dibutylmethacrylamide; caprolactone ring-opened adducts of 2-hydroxyethyl acrylate or methacrylate; (meth)acrylic esters of polyhydric alcohols; etc. Examples of the other ethylenic unsaturated monomers that can be copolymerized with the acrylic monomers include styrene, α-methylstyrene, itaconic acid, maleic acid, vinyl acetate, etc.

Examples of the polyester resins include oil-free polyester resins obtained by condensation of a polyhydric alcohol and a polybasic acid, and oil-modified polyester resins obtained by reacting a polyhydric alcohol and a polybasic acid with an oil component of one or more fatty acids of a castor oil, a dehydrated castor oil, a tung oil, a safflower oil, a soybean oil, a linseed oil, a tall oil, a coconut oil, etc.

As the crosslinking agent, an amino resin and/or a blocked polyisocyanate or polycarbodiimide compound may be used, and an amino resin may be more preferably used. Specific examples of the crosslinking agents include di-, tri-, tetra-, penta-, or hexa-methylolmelamines and alkyl ethers thereof, in which the alkyl group is methyl, ethyl, propyl, isopropyl, butyl, isobutyl, etc.; urea-formaldehyde condensation products; urea-melamine co-condensation products; etc. Melamine resins are more preferably used as the crosslinking agent.

The blocked polyisocyanate compound is a polyisocyanate compound blocked by a blocking agent. The blocking moiety in the blocked polyisocyanate compound is dissociated under a heating condition. Examples of the polyisocyanate compounds include aliphatic diisocyanates such as trimethylene diisocyanate, hexamethylene diisocyanate, and propylene diisocyanate; aromatic diisocyanates such as phenylene diisocyanate and naphthalene diisocyanate; aliphatic-aromatic isocyanates such as toluene diisocyanate and tolylene diisocyanate; tri- or more polyisocyanates such as triphenylmethane triisocyanate; dimers and trimers of tolylene diisocyanate; etc. Examples of the blocking agents include alcohols such as methyl alcohol and ethyl alcohol; tertiary amines such as diethanolamine; lactams such as caprolactam; oximes such as methyl ethyl ketoxime; etc.

The polycarbodiimide compound has at least two carbodiimide groups (-N=C=N- groups). Specific examples of the polycarbodiimide compounds include poly(4,4' -diphenylmethane carbodiimide), poly(3,3' -dimethyl-4,4' -biphenylmethane carbodiimide), poly(tolylcarbodiimide), poly(p-phenylene carbodiimide), poly(m-phenylene carbodiimide), poly(3,3' -dimethyl-4,4' -diphenylmethane carbodiimide), poly(naphthylene carbodiimide), poly(1,6-hexamethylene carbodiimide), poly(4,4' -methylene biscyclohexylcarbodiimide), poly(1,4-tetramethylene carbodiimide), poly(1,3-cyclohexylene carbodiimide), poly(1,4-cyclohexylene carbodiimide), poly(1,3-diisopropylphenylene carbodiimide), poly(1-methyl-3,5-diisopropylphenylene carbodiimide), poly(1,3,5-triethylphenylene carbodiimide), poly(triisopropylphenylene carbodiimide), etc.

In the vehicle of the aqueous first base coating composition, the mass ratio between the vehicle-forming resin and the crosslinking agent is such that the vehicle-forming resin content is 50 to 90% by mass and the crosslinking agent content is 10 to 50% by mass, more preferably such that the vehicle-forming resin content is 60 to 85% by mass and the crosslinking agent content is 15 to 40% by mass. When the crosslinking agent content is less than 10% by mass (or when the vehicle-forming resin content is more than 90% by mass), the crosslinking may be insufficient. On the other hand, when the crosslinking agent content is more than 50% by mass (or when the vehicle-forming resin content is less than 50% by mass), the storage stability of the coating composition is reduced and the curing rate is increased, thereby resulting in poor appearance of the coating.

The aqueous first base coating composition contains a brilliant pigment, and may further contain a color pigment and an extender pigment if necessary. The brilliant pigment preferably may include at least one brilliant pigment selected from the group consisting of an aluminum flake pigment, a metal oxide-coated alumina flake pigment, a metal oxide-coated silica flake pigment, a graphite pigment, an interference mica pigment, a color mica pigment, a metallic titanium flake pigment, a stainless steel flake pigment, an iron oxide plate pigment, a metal-plated glass flake pigment, a metal oxide-coated plated glass flake pigment, a hologram pigment, and a flake pigment composed of cholesteric liquid crystal polymers. The brilliant pigment may preferably comprises an aluminum flake pigment, a metal oxide-coated alumina flake pigment, a metal oxide-coated silica flake pigment, a graphite pigment, an interference mica pigment, a color mica pigment, a metallic titanium flake pigment, a stainless steel flake pigment, an iron oxide plate pigment, a metal-plated glass flake pigment, a metal oxide-coated plated glass flake pigment, a hologram pigment, a flake pigment composed of cholesteric liquid crystal polymers, or a combination thereof.

Examples of the color pigments include organic pigments such as an azo lake pigment, an insoluble azo pigment, a condensed azo pigment, a phthalocyanine pigment, an indigo pigment, a perynone pigment, a perylene pigment, a phthalone pigment, a dioxazine pigment, a quinacridon pigment, an iso-indolinone pigment, a benzimidazolone pigment, a diketopyrrolopyrrole pigment, and a metal complex pigment; and inorganic pigments such as iron oxide yellow, iron oxide red, carbon black, and titanium dioxide. Examples of the extender pigments include talc, calcium carbonate, precipitated barium sulfate, silica, etc.

The aqueous first base coating composition is generally provided in such a way that the above components are dissolved or dispersed in water (or deionized water) as a solvent (or dispersant). A composition comprising hydrophilic organic solvents substituting the water may also be included. In a mixture system of both water and organic solvents, the water content of the whole solvent may be from 51 to 100% by mass and the organic solvent content may be from 0 to 49% by mass, such that the water content may be higher than the organic solvent content.

The organic solvent may comprise such a solvent that is commonly used for the coating composition. Examples of the organic solvent may include hydrocarbons such as toluene and xylene; ketones such as acetone and methyl ethyl ketone; esters such as ethyl acetate, butyl acetate, cellosolve acetate, and butyl cellosolve; and alcohols. More preferred organic solvents include hydrophilic alcohol solvents.

Examples of the hydrophilic alcohol solvents may include methyl alcohol, ethyl alcohol, n-propyl alcohol, isopropyl alcohol, sec-butyl alcohol, tert-butyl alcohol, ethylene glycol, 1,2-propylene glycol, 1,3-butylene glycol, 2,3-butylene glycol, hexylene glycol, 2,5-hexanediol, dipropylene glycol, etc.

### Condition (A-3): Organic solvent/water ratio of solvent in aqueous first base coating composition

According to the present invention, in the method for forming a brilliant coating film with the proviso III, the solvent contained in the aqueous first base coating composition has the mass ratio of the organic solvent to the water (being referred to as "organic solvent/water ratio") from 5/95 to 49/51. When the organic solvent/water ratio is less than 5/95, the degree of dispersion of the components of the coating composition, particularly the brilliant pigment, may be reduced, thereby failing to achieve the splendid appearance. When the organic solvent/water ratio is more than 49/51, the VOC (volatile organic compound) content may be increased.

### Condition (B-3): Particular organic solvent for aqueous first base coating composition

According to the present invention, in the method for forming a brilliant coating film with the proviso III, the above organic solvent used for the solvent of the aqueous first brilliant base coating composition contains 40 to 100% by mass of a particular organic solvent. The particular organic solvent useful the present invention has an evaporation rate of 200 to 750 when n-butyl acetate has an evaporation rate of 100 at 25°C. Further, the particular organic solvent has a solubility parameter of 9,7 to 14.5.

When the evaporation rate of the particular organic solvent for the aqueous first base coating composition is less than 150, the particular organic solvent evaporates from the coating at a very low rate so that the dripping property and the appearance may be deteriorated. When the evaporation rate of the particular organic solvent is more than 800, the storage stability of the coating composition may be lowered due to the large volatilization volume. The evaporation rate of the particular organic solvent useful for the present invention is from 200 to 750.

When the solubility parameter of the particular organic solvent for the aqueous first base coating composition is less than 9.5, the particular organic solvent may be separated from the coating composition. When the solubility parameter is more than 14.5, the particular organic solvent is volatilized from the coating at a low rate. The solubility parameter of the particular organic solvent useful for the present invention is from 9.7 to 14.5.

The organic solvent(s) containing less than 40% by mass of the particular organic solvent is disadvantageous in that the orientation of the brilliant materials is worsened, etc. The organic solvent(s) preferably contains 50 to 100% by mass of the particular organic solvent.

The evaporation rate of the particular organic solvent is a relative value measured by a gravimetric method under the assumption that the evaporation rate of n-butyl acetate is 100 at 25°C, which is a value described in Paul Nylen, et al, *Modern Surface Coatings,* 1965. The solubility parameter of the particular organic solvent is determined based on values described in C. M. Hansen, *Ind. Eng. Chem. Prod. Res. Develop.,* 8[1]2 (1969).

The evaporation rates and the solubility parameters of typical organic solvents commonly used in the field of coating compositions are described below. The typical organic solvents include hydrocarbons such as toluene (evaporation rate 195, solubility parameter 8.9) and xylene (evaporation rate 68, solubility parameter 8.8); ketones such as acetone (evaporation rate 720, solubility parameter 9.8) and methyl ethyl ketone (evaporation rate 465, solubility parameter 9.3); esters such as ethyl acetate (evaporation rate 525, solubility parameter 9.1) and butyl acetate (evaporation rate 100, solubility parameter 8.5); and alcohols such as methyl alcohol (evaporation rate 370, solubility parameter 14.5), ethyl alcohol (evaporation rate 203, solubility parameter 13.0), isopropyl alcohol (evaporation rate 205, solubility parameter 11.5), n-butyl alcohol (evaporation rate 49, solubility parameter 11.3), propylene glycol (evaporation rate 1, solubility parameter 14.8), and 2-butoxyethanol (evaporation rate 10, solubility parameter 10.2).

The aqueous first base coating composition may contain an additive in addition to the above components, and examples of the additives include anti-precipitation agents, curing catalysts, ultraviolet absorbers, antioxidants, leveling agents, surface controlling agents such as silicones and organic polymers, anti-dripping agents, thickeners, defoaming agents, lubricants, and cross-linked polymer particles (or microgels).

### Step (2)

According to the present invention, in the step (2) of the method for forming a brilliant coating film, the second base coating is formed by applying the aqueous second brilliant base coating composition (which may be referred to as the aqueous second base coating composition) onto the first base coating formed in the step (1) at the second stage in the base coating zone.

The aqueous second base coating composition used in the second stage of the base coating zone may comprise the vehicle, the pigment, the solvent, and the additive usable for the aqueous first base coating composition.

### Condition (C): Organic solvent/water ratio of solvent in aqueous second base coating composition

According to an embodiment of the present invention, in the second method for forming a brilliant coating film, the brilliant coating film is formed under the condition (C) that the solvent contained in the aqueous second base coating composition has the organic solvent/water ratio of 5/95 to 49/51. Thus, the solvent of the aqueous second base coating composition has more water than the organic solvent. When the organic solvent/water mass ratio is less than 5/95, the degree of dispersion of the brilliant components of the coating composition may be lowered, thereby failing to achieve the splendid appearance. When the organic solvent/water mass ratio is more than 49/51, the composition is not so preferable in the viewpoint of the VOC. The organic solvent/water mass ratio may be more preferably from 10/90 to 45/55.

### Amount of fluorine- or silicone-based additive used in aqueous second base coating composition

According to an embodiment of the present invention, in the third method for forming a brilliant coating film, the aqueous second base coating composition contains 0.1 to 5 parts by mass of the fluorine- or silicone-based additive per 100 parts by mass of the vehicle solid contents, whereby the surface tension of the composition is reduced to improve the property of wetting with the aqueous first base coating.

Examples of the fluorine-based additives may include fluorinated alkyl carboxylates, fluorinated alkyl alkoxylates, and fluorinated alkyl esters.

Examples of the silicone-based additives may include polyether-modified polymethylalkylsiloxanes, polyether-modified polydimethylsiloxanes, polyester-modified polymethylalkylsiloxanes, silicone-modified polyacryls, and aralkyl-modified polymethylalkylsiloxanes.

When the amount of the fluorine- or silicone-based additive is less than 0.1 parts by mass per 100 parts by mass of the vehicle solid content, the surface tension may not be sufficiently reduced. When the amount is more than 5 parts by mass, the coating film performances may be deteriorated. The amount of the fluorine- or silicone-based additive is more preferably 0.2 to 2 parts by mass.

### Condition (A-1) : Solid contents of aqueous first and second base coating compositions

According to an embodiment of the present invention, in the method for forming a brilliant coating film with the proviso I, the aqueous first base coating composition has the solid content of 10 to 45% by mass, and the aqueous second base coating composition has the solid content of 10 to 40% by mass. When the solid content of the aqueous first base coating composition is less than 10% by mass, a larger amount of the composition is used to form the coating with a desired thickness, resulting in poor coating efficiency. When the solid content of the aqueous first base coating composition is more than 45% by mass, the appearance of the coating is deteriorated. The aqueous first base coating composition preferably has a solid content of 15 to 40% by mass. When the solid content of the aqueous second base coating composition is less than 10% by mass, a larger amount of the composition is used to form the coating with a desired thickness, resulting in poor coating efficiency. When the solid content of the aqueous second base coating composition is more than 40% by mass, the orientation of the brilliant pigments is deteriorated. The aqueous second base coating composition preferably has a solid content of 11 to 30% by mass. Each coating composition has the above solid content at the time the composition is applied, and the solid content is equal to a heating residue content obtained by heating the composition to remove the volatile components. In the present invention, the heating residue content is obtained from the difference between mass values of the coating composition measured before and after heating the composition at 105°C for 3 hours.

### Condition (B-1) : Solid content ratio between aqueous first and second base coating compositions

According to an embodiment of the present invention, in the method for forming a brilliant coating film with the proviso I, the solid content ratio of the solid content of the aqueous first base coating composition to that of the aqueous second base coating composition is from 1.1/1 to 4/1. Thus, the solid content of the aqueous first base coating composition is more than that of the aqueous second base coating composition. When the solid content ratio is not within the above range, the orientation of the brilliant pigments may be deteriorated. More preferably, the solid content ratio may be from 1.3/1 to 2.5/1.

### Condition (D): Dry film thickness ratio between aqueous first and second base coatings

According to the present invention, the dry film thickness ratio of the dry film thickness of the first base coating to that of the second base coating is from 1.5/1 to 5/1. Thus, the dry film thickness of the aqueous first base coating is larger than that of the aqueous second base coating. When the dry film thickness ratio between the first and second base coatings is less than 1.5/1, the orientation of the brilliant pigments may be deteriorated. If the dry film thickness ratio is more than 5/1, the brilliantness may become uneven. The dry film thickness ratio may be more preferably from 1.5/1 to 3/1.

The aqueous first base coating preferably has a dry film thickness of 5 to 15 µm, and the aqueous second base coating preferably has a dry film thickness of 2 to 8 µm.

### Condition (A-2) : Brilliant pigment PWCs of aqueous first and second base coating compositions

According to the present invention, in the method for forming a brilliant coating film with the proviso II, the aqueous first base coating composition has the brilliant pigment PWC of 3 to 25%, and the aqueous second base coating composition has the brilliant pigment PWC of 7 to 30%. When the brilliant pigment PWC of the aqueous first base coating composition is less than 1%, the hiding property may be insufficient. When the brilliant pigment PWC of the aqueous first base coating composition is more than 30%, the coating performance may be deteriorated. The aqueous first base coating composition has a brilliant pigment PWC of 3 to 25%. When the brilliant pigment PWC of the aqueous second base coating composition is less than 5%, the brilliantness may be insufficient. When the brilliant pigment PWC of the aqueous second base coating composition is more than 40%, the orientation of the brilliant pigments may be deteriorated to lower the coating appearance. The aqueous second base coating composition have a brilliant pigment PWC of 7 to 30%. The brilliant pigments preferably have a flip-flop property, which means that the reflection light intensity is changed depending on the observation angle (or the light-receiving angle).

### Condition (B-2) : Brilliant pigment PWC ratio between aqueous first and second base coating compositions

According to the present invention, in the method for forming a brilliant coating film with the proviso II, the brilliant pigment PWC ratio of the brilliant pigment PWC of the aqueous first base coating composition to that of the aqueous second base coating composition is from to. Thus, the brilliant pigment PWC of the aqueous second base coating composition is larger than that of the aqueous first base coating composition. If the brilliant pigment PWC ratio is less than 1/4, the brilliantness may become uneven. On the other hand, when the brilliant pigment PWC ratio is more than 1/1.1, the orientation of the brilliant pigments may be insufficient.

The aqueous first and second base coatings are preferably formed by a spray coating process. Specifically, the formed aqueous first base coating may be subjected to setting and then coated wet-on-wet with the aqueous second base coating. The formed aqueous second base coating may be subjected to setting for 2 minutes, and then preheated at 40 to 80°C for 1 to 10 minutes with a drying furnace if necessary, to obtain uncured base coatings.

A rotary atomizing-type bell-shaped coating apparatus or an air atomizing-type coating apparatus is preferably used as a spray gun in the spray coating process. For example, Metallic bell G1-COPES bell (ABB Industry Corp.) may be used as the rotary atomizing-type bell-shaped coating apparatus. When the rotary atomizing-type coating apparatus is used, the rotating speed may be preferably 2×10⁴ to 4×10⁴ rpm, and the discharge rate may be preferably 80 to 250 cc/min.

### Step (3)

According to of the present invention, in the step (3) of the method for forming a brilliant coating film, the clear coating is formed by applying the clear coating composition onto the aqueous second base coating formed in the step (2) in the clear coating zone.

In the step (3), the clear coating is formed on the uncured second base coating film obtained in the step (2) in the clear coating zone. The clear coating film may be a transparent colorless coating film that does not hide the base coating film, or a translucent, so-called colored clear coating film. Such a clear coating film as the top clear coating film is formed on the base coating films that the brilliantness may be improved and that projecting pigments from the base coating films may be covered with the clear coating film.

A coating composition that is usually used for overcoating may be used as the clear coating composition for the clear coating film. For example, a mixture of the above-mentioned crosslinking agent and at least one heat-curable resin selected from acrylic resins, polyester resins, fluororesins, epoxy resins, polyurethane resins, polyether resins, and modified resins thereof may be used as the clear coating composition. Further, at least one heat-curable resin, which may be mixed with the above-mentioned crosslinking agent, may be selected from the group consisting of acrylic resins, polyester resins, fluororesins, epoxy resins, polyurethane resins, polyether resins, and modified resins thereof such that a mixture of the selected resin and the agent may be used as the clear coating composition.

The clear coating composition can contain an additive such as a color pigment, an extender pigment, a modifying agent, an ultraviolet absorber, a leveling agent, a dispersing agent, and a defoaming agent, as long as the additive does not impair the transparency of the composition. A composition described in JP-B-8-19315, which contains a carboxyl-containing polymer and an epoxy-containing polymer, may be preferably used as the clear coating composition from the viewpoint of acid rain resistance. The clear coating composition may be an organic solvent type, an aqueous type, powder type, etc. The organic solvent or aqueous type clear coating composition may be a one-pack type composition or a two-pack type composition such as a two-pack urethane resin coating composition.

The clear coating film has a dry film thickness of 10 to 60 µm. When the dry film thickness is not within the range, there may be defects in the clear coating film appearance and disadvantages in the coating workability. The dry film thickness may be more preferably from 20 to 50 µm.

### Step (4)

According to of the present invention, in the step (4) of the first method for forming a brilliant coating film, the uncured coating film formed in the steps (1), (2) and (3) are simultaneously heated and cured.

The uncured coating film formed in the steps (1), (2) and (3) are dried or cured at a predetermined temperature for a predetermined period of time in a drying zone adjacent to the clear coating zone, to form the multilayered brilliant coating film on the substrate. The temperature and the period of time for drying or curing may be determined in accordance with the types of the aqueous first base coating composition, the aqueous second base coating composition, and the clear coating composition.

### Coated article

According to an embodiment of the present invention, the coated article comprises the brilliant coating film formed by any one of the first to fifth methods as described above. In the case of using the first method, the coated article comprises the brilliant coating film formed on the substrate in the steps (1) to (4) with at least the provisos II, and III. In the case of using the second method, the coated article comprises the brilliant coating film formed on the substrate under the condition (C) based on the first method. In the case of using the third method, the coated article comprises the brilliant coating film, which is formed on the substrate by using the aqueous second brilliant base coating composition containing 0.1 to 5 parts by mass of the fluorine- or silicone-based additive per 100 parts by mass of the vehicle solid contents, based on any one of the first to fourth methods.

The present invention will be described in more detail below with reference to Examples and Comparative Examples without intention of limiting the scope of the present invention. Unless otherwise noted, the amounts of components are shown as the mass ratio (parts by mass), and the trade names of raw materials, coating compositions, and apparatuses are used.

### Examples 1 to 16 and Comparative Examples 1 to 5

### Preparation of substrates 1 and 2

A dull steel plate having a length of 300 mm, a width of 100 mm, and a thickness of 0.8 mm was treated with zinc phosphate. Then, a cationic electrodeposition coating composition (POWERTOP V-50, Nippon Paint Co., Ltd.) was electrodeposited onto the dull steel plate and baked at 160°C for 30 minutes to obtain an electrodeposition coating film having a dry film thickness of 25 µm. An intermediate coating composition (ORGA P-5 Sealer, Nippon Paint Co., Ltd.) was applied onto the electrodeposition coating film by an air spray coating process and baked at 140°C for 30 minutes to form an intermediate coating film having a dry film thickness of 40 µm, whereby a substrate 1 was prepared.

A plastic polypropylene plate having a length of 300 mm, a width of 100 mm, and a thickness of 3.0 mm was washed and degreased. Then, the degreased plate was spray-coated with a primer (RB116 Primer, Nippon Bee Chemical Co., Ltd.) and dried at a surface temperature of 80°C for 10 minutes such that the film of the primer had a dry film thickness of 10 µm, whereby a substrate 2 was prepared.

### Step (1) : Formation of first base coating

An aqueous first base coating composition containing a brilliant pigment in an amount as shown in Table 1, which is divided into three parts (1), (2), and (3), and a necessary color pigment to be mixed was applied to the substrate 1 or 2 so as to form the first base coating with a dry film thickness as shown in Table 1 such that the substrate 1 or 2 was coated with the first base coating film at the first stage of a base coating zone. Here, the aqueous first base coating composition was prepared by using an acryl-melamine resin coating composition (AQUAREX AR2100, Nippon Paint Co., Ltd.) as a base material so that the properties of the base coating were controlled as shown in Table 1. In Example 11, on the other hand, an aqueous melamine-carbodiimide-acryl coating composition (KX-0077, Nippon Bee Chemical Co., Ltd.) was used as a base material.

### Step (2) : Formation of second base coating

After the aqueous first base coating was subjected to setting for 2 minutes, and an aqueous second base coating composition containing a brilliant pigment in an amount as shown in Table 1, a color pigment to be mixed as necessary, and an additive agent was applied thereon in a wet-on-wet condition at the second stage of the base coating zone such that the second base coating was formed with a dry film thickness as shown in Table 1. Here, the aqueous second base coating composition containing a brilliant pigment was prepared with an acryl-melamine resin coating composition (AQUAREX AR2100, Nippon Paint Co., Ltd.) as a base material such that the properties of the base coating were controlled as shown in Table 1. In Example 11, on the other hand, an aqueous melamine-carbodiimide-acryl coating composition (KX-0077, Nippon Bee Chemical Co., Ltd.) was used as a base material.

### Step (3) : Formation of clear coating (first brilliant coating film formation method)

The second base coating was subjected to setting for 2 minutes, preheated at 80°C for 3 minutes, and coated with the following clear coating composition in a clear coating zone such that the formed clear coating had a dry film thickness of 35 µm. A acrylic resin-based solution-type clear coating composition (SUPERLAC O-100 Clear, Nippon Paint Co., Ltd.) was used as a clear coating composition 1, and a solution-type clear coating composition composed of a blend of a carboxyl-containing polymer and an epoxy-containing polymer (MACFLOW O-330 Clear, Nippon Paint Co., Ltd.) was used as a clear coating composition 2. The substrate 2 was spray-coated with an acryl-urethane clear coating composition 3 (R290 Clear, Nippon Bee Chemical Co., Ltd.) such that the clear coating had a dry film thickness of 30 µm.

### Step (4) : Heat-curing of uncured coatings (first brilliant coating film formation method)

The clear coating was subjected to setting at the room temperature for 10 minutes, and baked at 140°C for 30 minutes. In the case of the substrate 2, the clear coating was subjected to setting at the room temperature for 10 minutes, and baked 80°C for 20 minutes. The brilliantness of thus-obtained multilayered coating film was evaluated by the following evaluation method. The results are shown in Table 1.

### Step (5) : Heat-curing of uncured coatings (second brilliant coating film formation method) : Example 12

The formed base coatings were baked at 140°C for 30 minutes. The brilliantness of thus-obtained multilayered coating film was evaluated by the following evaluation method. The results are shown in Table 1.

### Evaluation method

Finished appearance : A sample coating film was observed from approximately the front (a highlight portion) and from an approximately 15-degree angle (a shade portion) to evaluate visually the sparkling effect that shows the quality of the metallic coating film appearance and the appearance of the coating. The coating film which was observed less sparkling effect was evaluated as much better.
⊚ (*Excellent*): No sparkling effect. No uneven brilliantness or lowered orientation property were observed. The film had an excellent metallic finished appearance.
○ (*Good*): No sparkling effect. The film had a metallic finished appearance.
Δ (*Fair*): Sparkling effect on the shade portion.
× (*Poor*): Sparkling effect on both highlight and shade portions. The film had an ordinal metallic appearance. Uneven brilliantness or lowered orientation was observed.

FF effect (flip-flop effect) : Difference in brightness observed from between approximately the front (highlight portion) and the approximately 15-degree angle (shade portion) was evaluated. The flip-flop property may refer to difference in the reflection intensity as the observation angle (or the light-receiving angle) is changed.
⊚ (*Excellent*): Extremely large brightness difference between different angles.
○ (*Good*): Large brightness difference between different angles.
Δ (*Fair*): Small brightness difference between different angles.
× (*Pool*): Almost no brightness difference between different angles. An ordinal metallic appearance.

The following brilliant pigments, color pigments, and additives shown in Table 1 were used.

### Brilliant pigments

1: Aluminum flake pigment; Aluminum Paste MH-8801 (ASAHI KASEI CORPORATION).
2: Aluminum flake pigment; Aluminum Paste 91-0562 (TOYO ALUMINIUM K.K.).
3: Interference mica pigment; Xirallic T60-23WIII (Merck Ltd., Japan).

### Color pigments

1: Carbon black pigment; MA-100 (MITSUBISHI CHEMICAL CORPORATION).
2: Phthalocyanine blue pigment; Cyanine Blue G314 (SANYO COLOR WORKS, Ltd.).

### Additives

1: Fluorinated alkyl carboxylate; Florade FC-129 (SUMITOMO 3M LIMITED).
2: Organic modified polysiloxane; BYK-341 (BYK-Chemie JAPAN).

In Table 1 and following Tables 2 and 3 in the specification, each example or comparative example is described in Substrate, Brilliant pigment (Type and Amount(PWC)), Solvent, Solid content of coating composition, Dry film thickness, Organic solvent/water ratio, Solid content ratio between first and second coating compositions, Brilliant pigment PWC ratio between first and second coating compositions, Dry film thickness ratio between first and second coating films, Clear top coating composition, and Evaluations in Finished appearance and FF effect.

**Table 1 (1)**

| | | Substrate | First base coating | | | | |
|---|---|---|---|---|---|---|---|
| | | | Brilliant pigment | | Solvent | (A-1) Solid content of coating composition (%) | Dry film thickness (µm) |
| | | | Type | (A-2) Amount (PWC) | No (Table4) | | |
| Example | 1 | 1 | 1 | 15 | 1 | 20 | 6 |
| | 2 | 1 | 1 | 10 | 1 | 20 | 8 |
| | 3 | 1 | 2 | 10 | 1 | 20 | 8 |
| | 4 | 1 | 2 | 10 | 1 | 20 | 8 |
| | 5 | 1 | 3 | 10 | 1 | 20 | 8 |
| | 6 | 1 | 1 | 5 | 1 | 20 | 8 |
| | 7 | 1 | 1 | 10 | 1 | 30 | 8 |
| | 8 | 1 | 1 | 10 | 1 | 20 | 12 |
| | 9 | 1 | 2 | 10 | 1 | 20 | 8 |
| | 10 | 1 | 1 | 10 | 1 | 20 | 8 |
| | 11 | 2 | 1 | 10 | 1 | 20 | 8 |
| | 12 | 1 | 1 | 10 | 1 | 20 | 8 |
| | 13 | 1 | 1 | 10 | 1 | 20 | 8 |
| | 14 | 1 | 1 | 10 | 1 | 20 | 8 |
| | 15 | 1 | 1 | 10 | 1 | 11 | 8 |
| | 16 | 1 | 1 | 10 | 1 | 40 | 8 |
| Comparative Example | 1 | 1 | 1 | 15 | 7 | 20 | 6 |
| | 2 | 1 | 1 | 15 | 7 | 5 | 6 |
| | 3 | 1 | 1 | 15 | 7 | 50 | 6 |
| | 4 | 1 | 1 | 15 | 7 | 25 | 6 |
| | 5 | 1 | 1 | 15 | 7 | 20 | 6 |

**Table 1 (2)**

| | | Second base coating | | | | | | | |
|---|---|---|---|---|---|---|---|---|---|
| | | Brilliant pigment | | Other pigment | | Surfactant | | (A-1) Solid content of 9,7 coating composition (%) | Dry film thickness (*µ*m) |
| | | Type | (A-2) Amount (PWC) | Type | Amount (PWC) | Type | Amount (PHR) | | |
| Example | 1 | 1 | 15 | - | - | - | - | 15 | 6 |
| | 2 | 1 | 20 | - | - | - | - | 15 | 4 |
| | 3 | 1 | 20 | - | - | - | - | 15 | 4 |
| | 4 | 2 | 20 | - | - | - | - | 15 | 4 |
| | 5 | 3 | 20 | 2 | 5 | - | - | 15 | 4 |
| | 6 | 1 | 15 | - | - | - | - | 15 | 4 |
| | 7 | 1 | 20 | - | - | - | - | 15 | 4 |
| | 8 | 1 | 20 | - | - | - | - | 15 | 3 |
| | 9 | 2 | 2 0 | 1 | 2 | - | - | 15 | 4 |
| | 10 | 1 | 20 | - | - | - | - | 15 | 4 |
| | 11 | 1 | 20 | - | - | - | - | 15 | 4 |
| | 12 | 1 | 20 | - | - | - | - | 15 | 4 |
| | 13 | 1 | 20 | - | - | 1 | 0.5 | 15 | 4 |
| | 14 | 1 | 20 | - | - | 2 | 0.5 | 15 | 4 |
| | 15 | 1 | 20 | - | - | - | - | 10 | 4 |
| | 16 | 1 | 20 | - | - | - | - | 10 | 4 |
| Comparative Example | 1 | 1 | 15 | - | - | - | - | 20 | 6 |
| | 2 | 1 | 15 | - | - | - | - | 20 | 6 |
| | 3 | 1 | 15 | - | - | - | - | 2 0 | 6 |
| | 4 | 1 | 15 | - | - | - | - | 5 | 6 |
| | 5 | 1 | 15 | - | - | - | - | 45 | 6 |

**Table 1 (3)**

| | | (A-3) Organic solvent/water ratio of 9,7 first base coating composition | (B-1) Solid content ratio between first and second base coating compositions | (B-2) Brilliant pigment PWC ratio between first and second base coating compositions | (D) Dry film thickness ratio between first and second base coatings | Clear top coating | Evaluation results | |
|---|---|---|---|---|---|---|---|---|
| | | | | | | Coating composition | Finished appearance | FF effect |
| Example | 1 | 30/70 | 1.3/1 | 1/1 | 1/1 | 1 | ○ | ○ |
| | 2 | 30170 | 1.3/1 | 1/2 | 2/1 | 1 | ⊚ | ○ |
| | 3 | 30/70 | 1.3/1 | 1/2 | 2/1 | 1 | ⊚ | ○ |
| | 4 | 30/70 | 1.3/1 | 1/2 | 2/1 | 1 | ○ | ⊚ |
| | 5 | 30/70 | 1.3/1 | 1/2 | 2/1 | 1 | ○ | ○ |
| | 6 | 30/70 | 1.3/1 | 1/3 | 2/1 | 1 | ⊚ | ○ |
| | 7 | 30170 | 2/1 | 1/2 | 2/1 | 1 | ⊚ | ⊚ |
| | 8 | 30/70 | 1.3/1 | 1/2 | 4/1 | 1 | ○ | ⊚ |
| | 9 | 30/70 | 1.3/1 | 1/2 | 2/1 | 1 | ⊚ | ⊚ |
| | 10 | 30/70 | 1.3/1 | 1/2 | 2/1 | 2 | ⊚ | ○ |
| | 11 | 30/70 | 1.3/1 | 1/2 | 2/1 | 3 | ⊚ | ○ |
| | 12 | 30/70 | 1.3/1 | 1/2 | 2/1 | - | ⊚ | ○ |
| | 13 | 30/70 | 1.3/1 | 1/2 | 2/1 | 1 | ⊚ | ⊚ |
| | 14 | 30/70 | 1.3/1 | 1/2 | 2/1 | 1 | ⊚ | ⊚ |
| | 15 | 30/70 | 1.1/1 | 1/2 | 2/1 | 1 | ○ | ○ |
| | 16 | 30/70 | 4/1 | 1/2 | 2/1 | 1 | ⊚ | ○ |
| Comparative Example | 1 | 30/70 | 1/1 | 1/1 | 1/1 | 1 | × | Δ |
| | 2 | 30/70 | 0.3/1 | 1/1 | 1/1 | 1 | × | × |
| | 3 | 30/70 | 2.5/1 | 1/1 | 1/1 | 1 | × | × |
| | 4 | 30/70 | 5/1 | 1/1 | 1/1 | 1 | × | Δ |
| | 5 | 30/70 | 0.4/1 | 1/1 | 1/1 | 1 | × | × |

### Examples 17 to 30 and Comparative Examples 6 to 10

### Preparation of substrates 1 and 3

The substrates 1 and 2 were prepared in the same manner as Examples 1 to 16.

### Step (1) : Formation of first base coating

The substrate 1 or 2 was coated with an aqueous first base coating composition at the first stage of a base coating zone such that the first base coating had a dry film thickness as shown in Table 2, which is divided into three parts (1), (2), and (3). The aqueous first base coating composition contained an amount of a brilliant pigment shown in Table 2 and a necessary color pigment as required. Here, the aqueous first base coating composition was prepared with an acryl-melamine resin coating composition (AQUAREX AR2100, Nippon Paint Co., Ltd.) as a base material so that the properties of the base coating were controlled as shown in Table 2. In Example 27, on the other hand, an aqueous melamine-carbodiimide-acryl coating composition (KX-0077, Nippon Bee Chemical Co., Ltd.) was used as a base material.

### Step (2) : Formation of second base coating

After the first base coating was subjected to setting for 2 minutes, an aqueous second base coating composition containing the following kind of brilliant pigment as much as shown in Table 2, a necessary color pigment and a necessary additive was applied in a wet-on-wet condition at the second stage of the base coating zone such that the second base coating had a dry film thickness as shown in Table 2. Here, the aqueous second base coating composition was prepared with an acryl-melamine resin coating composition (AQUAREX AR2100, Nippon Paint Co., Ltd.) as a base material, such that the properties of the base coating were controlled as shown in Table 2. In Example 27, on the other hand, an aqueous melamine-carbodiimide-acryl coating composition (KX-0077, Nippon Bee Chemical Co., Ltd.) was used as a base material.

### Step (3) : Formation of clear coating (first brilliant coating film formation method)

The second base coating was subjected to setting for 2 minutes, preheated at 80°C for 3 minutes, and coated with the following clear coating composition in a clear coating zone such that the formed clear coating had a dry film thickness of 35 µm. A clear coating composition 1 : acrylic resin-based solution-type clear composition (SUPERLAC O-100 Clear, Nippon Paint Co., Ltd.) and a clear coating composition 2: a clear solution-type coating composition composed of a blend of a carboxyl-containing polymer and an epoxy-containing polymer (MACFLOW O-330 Clear, Nippon Paint Co., Ltd.) were used. The substrate 2 was spray-coated with an acryl-urethane coating composition (R290 Clear, Nippon Bee Chemical Co., Ltd.) such that the clear coating had a dry film thickness of 30 µm.

### Step (4): Heat-curing of uncured coatings (first brilliant coating film formation method)

The clear coating was subjected to setting at the room temperature for 10 minutes, and baked at 140°C for 30 minutes. In the case of using the substrate 3, the clear coating was subjected to setting at the room temperature for 10 minutes, and baked 80°C for 20 minutes. The brilliantness of thus-obtained multilayered coating film was evaluated in the same manner as employed with Examples 1 to 16. The results are shown in Table 2. The brilliant pigments, the color pigments, and the additives shown in Table 2 are identical to those used in Examples 1 to 16.

### Step (5) : Heat-curing of uncured coatings (second brilliant coating film formation method) : Example 28

The formed second base coating was subjected to setting at the room temperature for 10 minutes, and baked at 140°C for 30 minutes. The brilliantness of thus-obtained multilayered coating film was evaluated in the same manner as employed with Examples 1 to 16. The results are shown in Table 2.

**Table 2 (1)**

| | | Substrate | First base coating | | | | |
|---|---|---|---|---|---|---|---|
| | | | Brilliant pigment | | Solvent | (A-1) Solid content of 9,7 coating composition (%) | Dry film thickness (*µ*m) |
| | | | Type | (A-2) Amount (PWC) | No. (Table4) | | |
| Example | 17 | 1 | 1 | 6 | 1 | 23 | 6 |
| | 18 | 1 | 1 | 6 | 1 | 23 | 8 |
| | 19 | 1 | 2 | 6 | 1 | 23 | 8 |
| | 20 | 1 | 2 | 6 | 1 | 23 | 8 |
| | 21 | 1 | 1 | 6 | 1 | 23 | 8 |
| | 22 | 1 | 1 | 6 | 1 | 23 | 10 |
| | 23 | 1 | 1 | 2 | 1 | 23 | 8 |
| | 24 | 1 | 1 | 30 | 1 | 23 | 8 |
| | 25 | 1 | 1 | 6 | 1 | 23 | 8 |
| | 26 | 1 | 1 | 6 | 1 | 23 | 8 |
| | 27 | 2 | 1 | 6 | 1 | 23 | 8 |
| | 28 | 1 | 1 | 6 | 1 | 23 | 8 |
| | 29 | 1 | 1 | 6 | 1 | 23 | 8 |
| | 30 | 1 | 1 | 6 | 1 | 23 | 8 |
| Comparative Example | 6 | 1 | 1 | 15 | 7 | 23 | 6 |
| | 7 | 1 | 1 | 15 | 7 | 23 | 8 |
| | 8 | 1 | 1 | 0.5 | 7 | 23 | 8 |
| | 9 | 1 | 1 | 35 | 7 | 23 | 8 |
| | 10 | 1 | 1 | 15 | 7 | 23 | 8 |

**Table 2 (2)**

| | | Second base coating | | | | | | | |
|---|---|---|---|---|---|---|---|---|---|
| | | Brilliant pigment | | Other pigment | | Surfactant | | (A-1) Solid content of coating composition (%) | Dry film thickness (µm) |
| | | Type | (A-2) Amount (PWC) | Type | Amount (PWC) | Type | Amount (PHR) | | |
| Example | 17 | 1 | 18 | - | - | - | - | 16 | 6 |
| | 18 | 1 | 18 | - | - | - | - | 16 | 4 |
| | 19 | 1 | 18 | - | - | - | - | 16 | 4 |
| | 20 | 2 | 18 | - | - | - | - | 16 | 4 |
| | 21 | 1 | 18 | 2 | 5 | - | - | 16 | 4 |
| | 22 | 1 | 18 | - | - | - | - | 16 | 2 |
| | 23 | 1 | 8 | - | - | - | - | 16 | 4 |
| | 24 | 1 | 33 | - | - | - | - | 16 | 4 |
| | 25 | 1 | 18 | 1 | 2 | - | - | 16 | 4 |
| | 26 | 1 | 18 | - | - | - | - | 16 | 4 |
| | 27 | 1 | 18 | - | - | - | - | 16 | 4 |
| | 28 | 1 | 18 | - | - | - | - | 16 | 4 |
| | 29 | 1 | 18 | - | - | 1 | 0.5 | 16 | 4 |
| | 30 | 1 | 18 | - | - | 2 | 0.5 | 16 | 4 |
| Comparative Example | 6 | 1 | 15 | - | - | - | - | 23 | 6 |
| | 7 | 1 | 15 | - | - | - | - | 23 | 4 |
| | 8 | 1 | 2.5 | - | - | - | - | 23 | 4 |
| | 9 | 1 | 39 | - | - | - | - | 23 | 4 |
| | 10 | 1 | 45 | - | - | - | - | 23 | 4 |

**Table 2 (3)**

| | | (A-3) Organic solvent/water ratio of first base coating composition | (B-1) Solid content ratio between first and second base coating compositions | (B-2) Brilliant pigment PWC ratio between first and second base coating compositions | (D) Dry film thickness ratio between first and second base coatings | Clear top coating | Evaluation results | |
|---|---|---|---|---|---|---|---|---|
| | | | | | | Coating composition | Finished appearance | FF effect |
| Example | 17 | 30/70 | 1.4/1 | 1/3 | 1/1 | 1 | ○ | ○ |
| | 18 | 30/70 | 1.4/1 | 1/3 | 2/1 | 1 | ⊚ | ○ |
| | 19 | 30/70 | 1.4/1 | 1/3 | 2/1 | 1 | ○ | ○ |
| | 20 | 30/70 | 1.4/1 | 1/3 | 2/1 | 1 | ○ | ⊚ |
| | 21 | 30/70 | 1.4/1 | 1/3 | 2/1 | 1 | ⊚ | ○ |
| | 22 | 30/70 | 1.4/1 | 1/3 | 5/1 | 1 | ⊚ | ○ |
| | 23 | 30/70 | 1.4/1 | 1/4 | 2/1 | 1 | ○ | ⊚ |
| | 24 | 30/70 | 1.4/1 | 1/1.1 | 2/1 | 1 | ⊚ | ⊚ |
| | 25 | 30/70 | 1.4/1 | 1/3 | 2/1 | 1 | ⊚ | ⊚ |
| | 6 | 30/70 | 1.4/1 | 1/3 | 2/1 | 2 | ⊚ | ○ |
| | 27 | 30170 | 1.4/1 | 1/3 | 2/1 | 3 | ⊚ | ○ |
| | 28 | 30170 | 1.4/1 | 1/3 | 2/1 | - | ⊚ | ○ |
| | 29 | 30/70 | 1.4/1 | 1/3 | 2/1 | 1 | ⊚ | ⊚ |
| | 30 | 30/70 | 1.4/1 | 1/3 | 2/1 | 1 | ⊚ | ⊚ |
| Comparative Example | 6 | 30/70 | 1/1 | 1/1 | 1/1 | 1 | × | Δ |
| | 7 | 30/70 | 1/1 | 1/1 | 2/1 | 1 | Δ | Δ |
| | 8 | 30/70 | 1/1 | 1/5 | 2/1 | 1 | Δ | × |
| | 9 | 30/70 | 1/1 | 1/1.1 | 2/1 | 1 | × | Δ |
| | 10 | 30/70 | 1/1 | 1/3 | 2/1 | 1 | × | Δ |

### Examples 31 to 46 and Comparative Examples 11 to 14

### Preparation of substrates 1 and 2

The substrates 1 and 2 were prepared in the same manner as used in Examples 1 to 30.

### Step (1) : Formation of first base coating

The substrate 1 or 2 was coated with an aqueous first base coating composition at the first stage of a base coating zone such that the first base coating had a dry film thickness as shown in Table 3, which is divided into three parts (1), (2), and (3). The aqueous first base coating composition contained an amount of a brilliant pigment shown in Table 3 and a solvent as shown in Tables 3 and 4, and further contained a color pigment if necessary. The aqueous first base coating composition was prepared by using an acryl-melamine resin coating composition (AQUAREX AR2100, Nippon Paint Co., Ltd.) as a base material such that the properties of the base coating were controlled as shown in Table 3. In Example 43, on the other hand, an aqueous melamine-carbodiimide-acryl coating composition (KX-0077, Nippon Bee Chemical Co., Ltd.) was used as a base material.

Here, each solvent number in Table 4 is assigned by a composition thereof, which may comprise deionized water, methyl alcohol, isopropyl alcohol, acetone, 2-butoxy-ethan, xylen, toluene, or a combination thereof. Each organic component may be evaluated by the evaporation rate and solubility parameter as shown in Table 4. Each solvent is evaluated in the mass ratio of the particular organic solvent.

### Step (2) : Formation of second base coating

After the first base coating was subjected to setting for 2 minutes, an aqueous second base coating composition at the second stage of the base coating zone was applied in a wet-on-wet condition such that the second base coating had a dry film thickness as shown in Table 3. Here, the aqueous second base coating composition contained an amount of a brilliant pigment as shown in Table 3 and a solvent as shown in Tables 3 and 4 and a necessary color pigment and a necessary additive as required.

The aqueous second base coating composition was prepared with an acryl-melamine resin coating composition (AQUAREX AR2100, Nippon Paint Co., Ltd.) as a base material and the properties of the base coating were controlled as shown in Table 3. In Example 43, on the other hand, an aqueous melamine-carbodiimide-acryl coating composition (KX-0077, Nippon Bee Chemical Co., Ltd.) was used as a base material.

### Step (3) : Formation of clear coating (first brilliant coating film formation method)

The second base coating was subjected to setting for 3 minutes, preheated at 80°C for 3 minutes, and coated with the following clear coating composition in a clear coating zone such that the formed clear coating had a dry film thickness of 35 µm. A clear coating composition 1: an acrylic resin-based solution-type clear coating composition (SUPERLAC O-100 Clear, Nippon Paint Co., Ltd.) and a clear coating composition 2: a solution-type clear coating composition composed of a blend of a carboxyl-containing polymer and an epoxy-containing polymer (MACFLOW O-330 Clear, Nippon Paint Co., Ltd.) were used. The substrate 2 was spray-coated with an acryl-urethane clear coating composition (R290 Clear, Nippon Bee Chemical Co., Ltd.) such that the clear coating had a dry film thickness of 30 µm.

### Step (4) : Heat-curing of uncured coatings (first brilliant coating film formation method)

The clear coating was subjected to setting at the room temperature for 10 minutes, and baked at 140°C for 30 minutes. In the case of the substrate 2, the formed clear coating was subjected to setting at the room temperature for 10 minutes, and baked 80°C for 20 minutes. The brilliantness of thus-obtained multilayered coating film was evaluated in the same manner as employed in Examples 1 to 30. The results are shown in Table 3. The brilliant pigments, the color pigments, and the additives shown in Table 3 are identical to those used in Examples 1 to 30.

### Step (5) : Heat-curing of uncured coatings (second brilliant coating film formation method) : Example 44

The formed second base coating was subjected to setting at the room temperature for 10 minutes, and baked at 140°C for 30 minutes. The brilliantness of thus-obtained multilayered coating film was evaluated in the same manner as employed in Examples 1 to 30. The results are shown in Table 3.

**Table 3 (1)**

| | | Substrate | First base coating | | | | |
|---|---|---|---|---|---|---|---|
| | | | Brilliant pigment | | Solvent | (A-1) Solid content of 9,7 coating composition (%) | Dry film thickness (µm) |
| | | | Type | (A-2) Amount (PWC) | No. (Table 4) | | |
| Example | 31 | 1 | 1 | 15 | 1 | 24 | 6 |
| | 32 | 1 | 1 | 7 | 1 | 24 | 9 |
| | 33 | 1 | 2 | 7 | 1 | 24 | 9 |
| | 34 | 1 | 2 | 7 | 1 | 24 | 9 |
| | 35 | 1 | 3 | 7 | 1 | 24 | 9 |
| | 36 | 1 | 1 | 7 | 2 | 24 | 9 |
| | 37 | 1 | 1 | 7 | 3 | 24 | 9 |
| | 38 | 1 | 1 | 7 | 4 | 24 | 9 |
| | 39 | 1 | 1 | 7 | 1 | 30 | 9 |
| | 40 | 1 | 1 | 10 | 1 | 24 | 9 |
| | 41 | 1 | 1 | 7 | 1 | 24 | 9 |
| | 42 | 1 | 1 | 7 | 1 | 24 | 9 |
| | 43 | 2 | 1 | 7 | 1 | 24 | 9 |
| | 44 | 1 | 1 | 7 | 1 | 24 | 9 |
| | 45 | 1 | 1 | 7 | 1 | 24 | 9 |
| | 46 | 1 | 1 | 7 | 1 | 24 | 9 |
| Comparative Example | 11 | 1 | 1 | 15 | 5 | 24 | 6 |
| | 12 | 1 | 1 | 15 | 6 | 24 | 9 |
| | 13 | 1 | 1 | 15 | 7 | 24 | 9 |
| | 14 | 1 | 1 | 15 | 8 | 24 | 9 |

**Table 3 (2)**

| | | Second base coating | | | | | | | | |
|---|---|---|---|---|---|---|---|---|---|---|
| | | Brilliant pigment | | Color pigment | | Additive | | Solvent | (A-1) Solid content of coating composition (%) | Dry film thickness (µm) |
| | | Type | (A-2) Amount (PWC) | Type | Amount (PWC) | Type | Amount (PHR) | No. (Table 2) | | |
| Example | 31 | 1 | 15 | - | - | - | - | 5 | 24 | 6 |
| | 32 | 1 | 18 | - | - | - | - | 5 | 15 | 3 |
| | 33 | 1 | 18 | - | - | - | - | 5 | 15 | 3 |
| | 34 | 2 | 18 | - | - | - | - | 5 | 15 | 3 |
| | 35 | 3 | 18 | 2 | 5 | - | - | 5 | 15 | 3 |
| | 36 | 1 | 18 | - | - | - | - | 5 | 15 | 3 |
| | 37 | 1 | 18 | - | - | - | - | 5 | 15 | 3 |
| | 38 | 1 | 18 | - | - | - | - | 5 | 15 | 3 |
| | 39 | 1 | 18 | - | - | - | - | 5 | 15 | 3 |
| | 40 | 1 | 15 | - | - | - | - | 5 | 15 | 3 |
| | 41 | 1 | 18 | 1 | 2 | - | - | 5 | 15 | 3 |
| | 42 | 1 | 18 | - | - | - | - | 5 | 15 | 3 |
| | 43 | 1 | 18 | - | - | - | - | 5 | 15 | 3 |
| | 44 | 1 | 18 | - | - | - | - | 5 | 15 | 3 |
| | 45 | 1 | 18 | - | - | 1 | 0.5 | 5 | 15 | 3 |
| | 46 | 1 | 18 | - | - | - | - | 5 | 15 | 3 |
| Comparative Example | 11 | 1 | 15 | - | - | - | - | 5 | 24 | 6 |
| | 12 | 1 | 15 | - | - | - | - | 5 | 24 | 3 |
| | 13 | 1 | 15 | - | - | - | - | 5 | 24 | 3 |
| | 14 | 1 | 15 | - | - | - | - | 5 | 24 | 3 |

**Table 3 (3)**

| | | (A-3) Organic solvent/water ratio of first base coating composition | (B-1) Solid content ratio between first and second base coating compositions | (B-2)Brilliant pigment PWC ratio between first and second base coating compositions | (D) Dry film thickness ratio between first and second base coatings | Clear top coating | Evaluation results | |
|---|---|---|---|---|---|---|---|---|
| | | | | | | Coating composition | Finished appearance | FF effect |
| Example | 31 | 30/70 | 1/1 | 1/1 | 1/1 | 1 | ○ | ○ |
| | 32 | 30/70 | 1.6/1 | 1/2.6 | 3/1 | 1 | ⊚ | ○ |
| | 33 | 30/70 | 1.6/1 | 1/2.6 | 3/1 | 1 | ○ | ○ |
| | 34 | 30/70 | 1.6/1 | 1/2.6 | 3/1 | 1 | ○ | ⊚ |
| | 35 | 30/70 | 1.6/1 | 1/2.6 | 3/1 | 1 | ○ | ○ |
| | 36 | 30/70 | 1.6/1 | 1/2.6 | 3/1 | 1 | ⊚ | ⊚ |
| | 37 | 30/70 | 1.6/1 | 1/2.6 | 3/1 | 1 | ○ | ○ |
| | 38 | 15/85 | 1.6/1 | 1/2.6 | 3/1 | 1 | ○ | ○ |
| | 39 | 30/70 | 2/1 | 1/2.6 | 3/1 | 1 | ⊚ | ○ |
| | 40 | 30/70 | 1.6/1 | 1/1.5 | 3/1 | 1 | ⊚ | ○ |
| | 41 | 30/70 | 1.6/1 | 1/2.6 | 3/1 | 1 | ⊚ | ⊚ |
| | 42 | 30/70 | 1.6/1 | 1/2.6 | 3/1 | 2 | ⊚ | ○ |
| | 43 | 30/70 | 1.6/1 | 1/2.6 | 3/1 | 3 | ⊚ | ⊚ |
| | 44 | 30/70 | 1,6/1 | 1/2.6 | 3/1 | - | ⊚ | ⊚ |
| | 45 | 30/70 | 1.6/1 | 1/2.6 | 3/1 | 1 | ⊚ | ⊚ |
| | 46 | 5/95 | 1.6/1 | 1/2.6 | 3/1 | 1 | ○ | ⊚ |
| Comparative Example | 11 | 10/90 | 1/1 | 1/1 | 1/1 | 1 | × | Δ |
| | 12 | 2/98 | 1/1 | 1/1 | 3/1 | 1 | × | × |
| | 13 | 30/70 | 1/1 | 1/1 | 3/1 | 1 | × | × |
| | 14 | 30/70 | 1/1 | 1/1 | 3/1 | 1 | × | Δ |

**Table 4**

| Evaporation rate | - | 370 | 205 | 720 | 10 | 68 | 195 | Total | (B-3) Mass ratio (% by mass) of particular organic solvent having evaporation rate of 150 to 800 and solubility parameter of 9.5 to 14.5 to organic solvents for base coating composition |
|---|---|---|---|---|---|---|---|---|---|
| Solubility parameter | 23.4 | 14.5 | 11.5 | 9.8 | 10.2 | 8.8 | 8.9 | | |
| Solvent No. | Deionized water | Methyl alcohol | Isopropyl alcohol | Acetone | 2-Butoxyethanol | Xylene | Toluene | | |
| 1 | 70 | 18 | 0 | 0 | 12 | 0 | 0 | 100 | 60 |
| 2 | 70 | 0 | 24 | 0 | 6 | 0 | 0 | 100 | 80 |
| 3 | 70 | 0 | 0 | 15 | 15 | 0 | 0 | 100 | 50 |
| 4 | 85 | 0 | 9 | 0 | 6 | 0 | 0 | 100 | 60 |
| 5 | 90 | 0 | 2 | 0 | 7 | 1 | 0 | 100 | 20 |
| 6 | 98 | 0 | 0 | 0 | 2 | 0 | 0 | 100 | 0 |
| 7 | 70 | 0 | 3 | 0 | 12 | 15 | 0 | 100 | 10 |
| 8 | 70 | 0 | 3 | 0 | 12 | 0 | 15 | 100 | 10 |

As shown in Tables 1 to 3, the brilliant coating films of the Examples formed by the methods according to the embodiments of the present invention had almost no grain-like surface finish, a metallic appearance without uneven brightness by the aluminum flake pigment, etc. having metallic luster, and an improved flip-flop property by the interference mica pigment, etc. On the other hand, the films of Comparative Examples did not show the advantageous effects.

According to of the present invention, the formed multilayered brilliant coating films may have excellent brightness or brilliantness such that they may be more preferably used in the field where the brilliantness is preferable such as outer shells of the automobile and motorcycle, and parts of the automobile (wheels, bumpers, etc.).

The present application discloses the following items:
1. A method for forming a brilliant coating film on a substrate, comprising the steps of:
   (1) applying an aqueous first brilliant base coating composition to the substrate to form a first base coating at a first stage in a base coating zone;
   (2) applying an aqueous second brilliant base coating composition to the first base coating to form a second base coating at a second stage in the base coating zone;
   (3) applying a clear coating composition to the second base coating formed in the step (2) to form a clear coating in a clear coating zone; and
   (4) simultaneously heating the uncured coatings formed in the steps (1), (2) and (3) to cure the coatings,
   with at least provisos, II, and III, and optionally with proviso I
   the proviso I of a condition (A-1) that the aqueous first brilliant base coating composition has a solid content of 10 to 45% by mass and the aqueous second brilliant base coating composition has a solid content of 10 to 40% by mass, and a condition (B-1) that the ratio of the solid content of the aqueous first brilliant base coating composition to the solid content of the aqueous second brilliant base coating composition is 1.1/1 to 4/1;
   the proviso II of a condition (A-2) that the aqueous first brilliant base coating composition has a brilliant pigment mass concentration of 3 to 25% and the aqueous second brilliant base coating composition has a brilliant pigment mass concentration of 7 to 30%, and a condition (B-2) that the ratio of the brilliant pigment mass concentration of the aqueous first brilliant base coating composition to the brilliant pigment mass concentration of the aqueous second brilliant base coating composition is 1/3,5 to 1/1
   the proviso III of a condition (A-3) that the aqueous first brilliant base coating composition comprises at least one organic solvent and water, and the mass ratio of the at least one organic solvent to the water is from 5/95 to 49/51, and a condition (B-3) that the at least one organic solvent includes 40 to 100% by mass of a particular organic solvent, which has a solubility parameter of 9,7 to 14.5 and an evaporation rate of 200 to 750 when n-butyl acetate has an evaporation rate of 100 at 25°C. and
   the aqueous first base coating having a dry film thickness of 5 to 15 µm
   the aqueous second base coating having a dry film thickness of 2 to 8 µm
   the ratio of the dry film thickness of the first base coating to the dry film thickness of the second base coating being 1.5/1 to 5/1 and
   the clear coating film having a dry film thickness of 10 to 60 µm
2. The method for forming a brilliant coating film according to item 1, wherein the method satisfies a condition (C) that the aqueous second brilliant base coating composition comprises at least one organic solvent and water, and the mass ratio of the at least one organic solvent to the water is from 5/95 to 49/51.

The method for forming a brilliant coating film according to items 1 or 2, wherein the aqueous second brilliant base coating composition contains 0.1 to 5 parts by mass of a fluorine- or silicone-based additive per 100 parts by mass of a vehicle solid content.

A coated article comprising a brilliant coating film formed by the method according to any one of items 1 to 3.

## Claims

1. A method for forming a brilliant coating film on a substrate, comprising the steps of:
(1) applying an aqueous first brilliant base coating composition containing a brilliant pigment to the substrate to form a first base coating at a first stage in a base coating zone;
(2) applying, successively to applying the aqueous first brilliant base coating composition, an aqueous second brilliant base coating composition containing a brilliant pigment to the first base coating formed in the step (1) to form a second base coating at a second stage in the base coating zone without preheating the applied first base coating composition;
(3) applying a clear coating composition to the second base coating formed in the step (2) to form a clear coating in a clear coating zone; and
(4) simultaneously heating the uncured coatings formed in the steps (1), (2) and (3) to cure the coatings,
with the following proviso II:
the proviso II of a condition (A-2) that the aqueous first brilliant base coating composition has a brilliant pigment mass concentration of 3 to 25 % and the aqueous second brilliant base coating composition has a brilliant pigment mass concentration of 7 to 30%, and a condition (B-2) that the ratio of the brilliant pigment mass concentration of the aqueous first brilliant base coating composition to the brilliant pigment mass concentration of the aqueous second brilliant base coating composition is 1/3.5 to 1/1.5;
and with the following proviso III:
the proviso III of a condition (A-3) that the aqueous first brilliant base coating composition comprises at least one organic solvent and water, and the mass ratio of the at least one organic solvent to the water is from 5/95 to 49/51, and a condition (B-3) that the at least organic solvent includes 40 to 100% by mass of a particular organic solvent, which is acetone, methyl alcohol, ethyl alcohol, or isopropyl alcohol, and
the aqueous first base coating having a dry film thickness of 5 to 15 µm
the aqueous second base coating having a dry film thickness of 2 to 8 µm
the ratio of the dry film thickness of the first base coating to the dry film thickness of the second base coating being 1.5/1 to 5/1 and
the clear coating film having a dry film thickness of 10 to 60 µm.

2. The method for forming a brilliant coating film according to claim 1, wherein the brilliant pigment is at least one selected from the group consisting of an aluminium flake pigment, a metal oxide-coated alumina pigment, a metal oxide-coated silica flake pigment, a graphite pigment, an interference mica pigment, a color mica pigment, a metallic titanium flake pigment, a stainless steel flake pigment, an iron oxide plate pigment, a metal-plated glass flake pigment, a metal oxide-coated plated glass flake pigment, and a hologram pigment.

3. The method for forming a brilliant coating film according to claims 1 or 2, wherein the aqueous second brilliant base coating composition contains 0.1 to 5 parts by mass of a fluorine- or silicone-based additive per 100 parts by mass of a vehicle solid content.

4. A coated article comprising a brilliant coating film formed by the method according to any one of claims 1 to 3.

## Patentansprüche

1. Verfahren zur Herstellung eines Brillant-Beschichtungsfilms auf einem Substrat, umfassend die folgenden Schritte:
(1) Aufbringen einer wässrigen ersten Brillant-Basisbeschichtungszusammensetzung, welche ein Brillantpigment enthält, auf das Substrat, um bei einer ersten Stufe in einer Basisbeschichtungszone eine erste Basisbeschichtung auszubilden;
(2) Aufbringen, dem Aufbringen der wässrigen ersten Brillant-Basisbeschichtungszusammensetzung folgend, einer wässrigen zweiten Brillant-Basisbeschichtungszusammensetzung, welche ein Brillantpigment enthält, auf die erste Basisbeschichtung, welche in dem Schritt (1) ausgebildet worden ist, um bei einer zweiten Stufe in der Basisbeschichtungszone eine zweite Basisbeschichtung auszubilden, ohne die aufgebrachte erste Basisbeschichtungszusammensetzung vorzuwärmen;
(3) Aufbringen einer klaren Beschichtungszusammensetzung auf die zweite Basisbeschichtung, welche in dem Schritt (2) ausgebildet worden ist, um in einer klaren Beschichtungszone eine klare Beschichtung auszubilden; und
(4) Gleichzeitiges Erwärmen der ungehärteten Beschichtungen, welche in den Schritten (1), (2) und (3) ausgebildet worden sind, um die Beschichtungen zu härten,
mit der folgenden Maßgabe II:
der Maßgabe II einer Bedingung (A-2), dass die wässrige erste Brillant-Basisbeschichtungszusammensetzung eine Brillantpigment-Massenkonzentration von 3 bis 25 % aufweist und die wässrige zweite Brillant-Basisbeschichtungszusammensetzung eine Brillantpigment-Massenkonzentration von 7 bis 30% aufweist, und einer Bedingung (B-2), dass das Verhältnis der Brillantpigment-Massenkonzentration der wässrigen ersten Brillant-Basisbeschichtungszusammensetzung zu der Brillantpigment-Massenkonzentration der wässrigen zweiten Brillant-Basisbeschichtungszusammensetzung 1/3,5 bis 1/1,5 beträgt,
und mit der folgenden Maßgabe III:
der Maßgabe III einer Bedingung (A-3), dass die wässrige erste Brillant-Basisbeschichtungszusammensetzung wenigstens ein organisches Lösungsmittel und Wasser umfasst, und das Massenverhältnis des wenigstens einen organischen Lösungsmittel zu dem Wasser von 5/95 bis 49/51 beträgt, und einer Bedingung (B-3), dass das wenigstens eine organische Lösungsmittel 40 bis 100 Massen-% eines bestimmten organischen Lösungsmittels umfasst, welches Aceton, Methylalkohol, Ethylalkohol oder Isopropylalkohol ist, und
wobei die wässrige erste Basisbeschichtung eine Trockenfilmdicke von 5 bis 15 µm aufweist,
die wässrige zweite Basisbeschichtung eine Trockenfilmdicke von 2 bis 8 µm aufweist,
das Verhältnis der Trockenfilmdicke der ersten Basisbeschichtung zu der Trockenfilmdicke der zweiten Basisbeschichtung 1,5/1 bis 5/1 beträgt
und der klare Beschichtungsfilm eine Trockenfilmdicke von 10 bis 60 µm aufweist.

2. Verfahren zur Herstellung eines Brillant-Beschichtungsfilms nach Anspruch 1, wobei das Brillantpigment wenigstens eines ist, welches aus der Gruppe ausgewählt ist, bestehend aus einem Aluminiumflockenpigment, einem metalloxidbeschichteten Aluminiumoxid-Pigment, einem metalloxidbeschichteten Siliziumdioxid-Flockenpigment, einem Graphitpigment, einem Interferenzglimmerpigment, einem Farbglimmerpigment, einem metallischen Titan-Flockenpigment, einem Flockenpigment aus nichtrostendem Stahl, einem Eisenoxid-Plattenpigment, einem metallplattierten Glas-Flockenpigment, einem metalloxidbeschichteten plattierten Glas-Flockenpigment und einem Hologrammpigment.

3. Verfahren zur Herstellung eines Brillant-Beschichtungsfilms nach Anspruch 1 oder 2, wobei die wässrige zweite Brillant-Basisbeschichtungszusammensetzung 0,1 bis 5 Masseteile eines auf Fluor oder Silikon basierenden Additivs pro 100 Masseteilen eines Vehikelfeststoffgehalts enthält.

4. Beschichteter Artikel, welcher einen Brillant-Beschichtungsfilm umfasst, welcher durch das Verfahren gemäß einem der Ansprüche 1 bis 3 hergestellt ist.

## Revendications

1. Procédé de formation d'un film de revêtement brillant sur un substrat, comprenant les étapes de :
(1) application d'une première composition de revêtement de base brillant aqueux contenant un pigment brillant au substrat pour former un premier revêtement de base à un premier stade dans une zone de revêtement de base ;
(2) application, successivement à l'application de la première composition de revêtement de base brillant aqueux, d'une seconde composition de revêtement de base brillant aqueux contenant un pigment brillant au premier revêtement de base formé à l'étape (1) pour former un second revêtement de base à un second stade dans la zone de revêtement de base, sans préchauffer la première composition de revêtement de base appliquée ;
(3) application d'une composition de revêtement transparent au second revêtement de base formé à l'étape (2) pour former un revêtement transparent dans une zone de revêtement transparent ; et
(4) chauffage simultané des revêtements non durcis formés aux étapes (1), (2) et (3) pour durcir les revêtements,
avec la réserve II suivante :
la réserve II d'une condition (A-2) selon laquelle la première composition de revêtement de base brillant aqueux a une concentration en masse en pigment brillant de 3 à 25 % et la seconde composition de revêtement de base brillant aqueux a une concentration en masse en pigment brillant de 7 à 30 %, et d'une condition (B-2) selon laquelle un rapport entre la concentration en masse en pigment brillant de la première composition de revêtement de base brillant aqueux et la concentration en masse en pigment brillant de la seconde composition de revêtement de base brillant aqueux est de 1/3,5 à 1/1,5 ;
et avec la réserve III suivante :
la réserve III d'une condition (A-3) selon laquelle la première composition de revêtement de base brillant aqueux comprend au moins un solvant organique et de l'eau, et le rapport en masse entre l'au moins un solvant organique et l'eau est de 5/95 à 49/51, et d'une condition (B-3) selon laquelle l'au moins un solvant organique comporte 40 à 100 % en masse d'un solvant organique particulier, qui est l'acétone, l'alcool méthylique, l'alcool éthylique, ou l'alcool isopropylique, et
le premier revêtement de base aqueux ayant une épaisseur de film sec de 5 à 15 µm le second revêtement de base aqueux ayant une épaisseur de film sec de 2 à 8 µm le rapport entre l'épaisseur de film sec du premier revêtement de base et l'épaisseur de film sec du second revêtement de base étant de 1,5/1 à 5/1 et
le film de revêtement transparent ayant une épaisseur de film sec de 10 à 60 µm.

2. Procédé de formation d'un film de revêtement brillant selon la revendication 1, dans lequel le pigment brillant est au moins un élément choisi dans le groupe consistant en un pigment lamellaire d'aluminium, un pigment d'alumine revêtu d'oxyde de métal, un pigment lamellaire de silice revêtu d'oxyde de métal, un pigment de graphite, un pigment interférentiel de mica, un pigment de mica coloré, un pigment lamellaire de titane métallique, un pigment lamellaire d'acier inoxydable, un pigment en plaque d'oxyde de fer, un pigment lamellaire de verre plaqué de métal, un pigment lamellaire de verre plaqué et revêtu d'oxyde de métal, et un pigment d'hologramme.

3. Procédé de formation d'un film de revêtement brillant selon l'une quelconque des revendications 1 ou 2, dans lequel la seconde composition de revêtement de base brillant aqueux contient de 0,1 à 5 parties en masse d'un additif à base de fluor ou de silicone pour 100 parties en masse d'une teneur en matière sèche de milieu de suspension.

4. Article revêtu comprenant un film de revêtement brillant formé par le procédé selon l'une quelconque des revendications 1 à 3.
